

1

3,206,384

## PROCESS FOR PRODUCING CORROSION RESISTANT COATING OF BARIUM FERRATE ON FERROUS METALS

Paul H. Margulies, Princeton, and William J. Tillis, Levittown, N.J., assignors to FMC Corporation, a corporation of Delaware

No Drawing. Filed Apr. 24, 1961, Ser. No. 104,780  
7 Claims. (Cl. 204—56)

This invention relates to the production of a resistant coating on ferrous metals, and more particularly to the application of a ferrate coating on the surfaces of ferrous metals.

Many methods are available for preventing corrosion of ferrous metal surfaces. The most popular commercial method involves placing a "conversion coating" on the surface of the ferrous metal to insulate it from a corrosive atmosphere. These "conversion coatings" result from the deposition of metal compounds on the surface of the workpiece.

One of these "conversion coatings" which is of interest for preventing corrosion of ferrous metals is the "ferrate film." Ferrate films have been produced on ferrous metal surfaces in the past by maintaining the ferrous metal surface (or other metal surface) in a bath of sodium or potassium ferrate for about 1 hour. These soluble ferrates, e.g., sodium ferrate, exist in solution in an unstable condition and deposit on the immersed workpiece, leaving a thin yellow coat of sodium ferrate ( $\text{Na}_2\text{FeO}_4$ ). This process is disclosed in U.S. Patent No. 2,850,416, issued to John E. Castle on September 2, 1958.

While these films afford some measure of corrosion resistance, the method of application as well as the degree of corrosion protection afforded by these films has not been commercially acceptable. The use of unstable solutions requiring freshly made chemicals, and the lengthy time for producing the film is a serious drawback when this process is sought to be commercially exploited. Moreover, the sodium ferrate or potassium ferrate which is deposited on the workpiece, does not give high corrosion resistance vis-a-vis other commercial conversion coatings, e.g., phosphate coatings. Another drawback to this process is that it permits only soluble ferrate salts to be employed even though other ferrates are known, since the ferrate must form on the workpiece from a prepared solution of the ferrate. Obviously insoluble ferrates cannot be employed, since they cannot be dissolved.

It is an object of the present invention to form a corrosion resistant, insoluble ferrate coating in-situ on the surface of ferrous metals from a stable liquid solution, in a short time.

These and other objects will be apparent from the following description.

It has now been determined, quite unexpectedly, that corrosion resistant films of barium ferrate ( $\text{BaFeO}_4$ ) can be formed in-situ on the surfaces of ferrous metals, by anodic treatment of these ferrous metals while in an alkaline solution of a soluble barium salt, a barium hydroxide or a barium oxide; the alkaline solution of barium salt, a barium hydroxide or a barium oxide serves as the electrolyte and filming bath, the ferrous workpiece serves as the anode, and a conductor serves as the cathode.

The one-formation of an insoluble barium ferrate in-situ on the surface of the anodic workpiece is quite un-

2

expected, since the prior process required all the reagents, including the iron which goes into the coating as well as the soluble sodium or potassium salt, to be dissolved in the treating solution. By contrast, the present process only uses an alkaline solution of a soluble barium salt, a barium hydroxide or a barium oxide, the iron in the coating being supplied by the anodic ferrous workpiece. The insoluble barium ferrate compound which results is formed in-situ at the surface of the ferrous anode and instantly deposits on this surface as an adherent, corrosion resistant layer. The barium ferrate layer is highly effective as a corrosion resistant surface, being more resistant than certain commercial conversion coatings such as iron phosphates, and offering corrosion resistance at least equal to commercially employed phosphate coatings, such as zinc phosphate.

In the operation of the present process an alkaline solution of a barium salt, a barium hydroxide or a barium oxide, preferably in a concentration of  $\frac{1}{2}$  N or above, constitutes the electrolyte. The maximum allowable concentration of a barium salt, a barium hydroxide or a barium oxide which may be employed is limited only by the solubility of the compound in solution. The barium compound which has been found most useful is  $\text{Ba}(\text{OH})_2 \cdot 8\text{H}_2\text{O}$ , although barium oxide, hydrated barium oxides, and anhydrous barium hydroxide can be employed. Soluble barium salts such as barium acetate, barium nitrate, and barium chloride, are also effective when used in alkaline solutions. The barium salt, barium hydroxide or barium oxide solution will yield barium ferrate per se, by anodic treatment of a ferrous workpiece, as long as the barium solution is alkaline. However, in order for the production of a corrosion resistant film of the newly formed barium ferrate on the surface of anodic workpiece, the barium salt, barium hydroxide or barium oxide solution must have a high alkalinity. In general, the corrosion resistance of the barium ferrate film increases with higher alkalinity until an optimum alkalinity is reached. It has been found that uniform films of  $\text{BaFeO}_4$  having good corrosion resistance are obtained with barium salt, barium hydroxide or barium oxide solutions having pH's of about 12.5 and above. The films obtained at lower pH values tend to be thinner and to be non-uniform. While these latter films also offer some measure of corrosion resistance and can be used in this application, they have not been found to be as efficacious as the films produced from barium salt, barium hydroxide or barium oxide solutions having pH's of about 12.5 and above.

The film-producing electrolyte may be made up using  $\text{Ba}(\text{OH})_2$  alone, or mixed with an alkali metal hydroxide. When  $\text{Ba}(\text{OH})_2$  is used alone, a solution in the range of  $\frac{1}{2}$  N to about 1 N should be employed since solutions containing more than 1 N  $\text{Ba}(\text{OH})_2$  exceed the practical solubility limits and are wasteful of barium, while concentrations below  $\frac{1}{2}$  N result in films which are too thin for completely adequate corrosion protection. The addition of an alkali metal hydroxide to the barium solution is the preferred method of operation since more uniform coatings are obtained with this electrolyte. The alkali metal hydroxide, e.g.,  $\text{NaOH}$  or  $\text{KOH}$ , is added within the range of 0.5 N to 7.5 N, to a 1 N solution of  $\text{Ba}(\text{OH})_2$ . When an alkali metal hydroxide is added to the electrolyte an additional advantage is obtained, over and above that of obtaining more uniform coatings. This is in the

lowering of the minimum concentration of barium salt from  $\frac{1}{5}$  N to as low as  $\frac{1}{20}$  N, required for the successful production of coatings. An electrolyte containing about 5 N NaOH and about 1 N Ba(OH)<sub>2</sub> has been found most suitable.

The ferrous metal workpiece to be coated is placed within the electrolyte, and is connected to a source of direct current. The ferrous object constitutes the anode, while a metallic conductor which is resistant to the electrolyte serves as the cathode e.g. steel sheets, carbon, platinum. If desired a suitable metal container used to hold the electrolyte solution can constitute the cathode.

A potential of at least about 1.4 volts must be applied before film formation begins. Films of barium ferrate will form at all potentials above about 1.4 volts. The minimum current which is required to produce these films is about 2 amperes per square foot of anodic surface (a.s.f.). The exact amount of current which can be employed depends upon factors such as voltage and internal resistance of the cell. Currents as high as 360 a.s.f. have been employed successfully.

Barium ferrate films which are applied to ferrous metal surfaces at from about 2 to about 4 volts exhibit good resistance against surface corrosion. The films may be applied at potentials of 2 volts with only about 5 to 20 a.s.f. At potentials of about 4 volts, a.s.f. values of about 144 have been found to give good results. Coatings prepared for the same length of time, at about 2 volts and at about 4 volts, are virtually identical except that those prepared at about 2 volts appear to have a more uniform surface when subject to a microscopic examination.

While the exact reason for the deposition of a more uniform coating at low electromotive potentials is not known, it is believed due to the less rapid formation of micro-bubbles at 2 volts than at 4 volts, which results in little or no microsized irregularities on the surface of the film. Nevertheless, films deposited at the higher potentials offer good corrosion resistance against corrosive atmospheres, while those deposited at lower potentials offer good resistance against both corrosive atmospheres and water immersion.

The films of the present process can be formed with the electrolytic bath at temperatures of about 160° to 220° F. At these temperatures the film begins depositing as soon as current is applied. The preferred time and temperatures have been found to be about 1 to 12 minutes and about 180° to 190° F. The temperature of the filming electrolyte, and the time of deposition, are extremely important since the thickness of the film which deposits on the ferrous metal surface is dependent upon both of these variables. The thickness of the film increases with higher temperatures and with longer deposition periods.

The films which are produced at 2 volts are not as thick as those applied at 4 volts under identical condition. However, since the thickness of the film is dependent upon both the treating time and the temperature of the electrolyte, it is possible to obtain the desirably uniform films produced at about 2 volts without sacrificing film thickness, either by increasing the temperature of the

electrolyte bath, or by increasing the filming time. For example, when employing an electrolyte at about 180° F., and applying 4 volts for 4 minutes, a barium ferrate coating weighing 206 mg./ft.<sup>2</sup> is obtained; if only 2 volts are applied for 4 minutes, but the electrolyte is raised to a temperature of 194° F., the same weight of barium ferrate coating is obtained as in the previous case.

By means of the present process, and by employing a coating time of only 4 minutes, 100 gallons of electrolyte containing 1 N Ba(OH)<sub>2</sub> can uniformly coat, on a conservative basis, over 10,000 square feet of ferrous metal surface. With respect to the power requirement, a potential of 4 volts applied with 144 a.s.f. of anode surface for 4 minutes, requires 0.0385 kilowatt hour for filming each square foot. If a potential of 2 volts at 15 a.s.f. of anode surface is employed for 4 minutes, only 0.002 kilowatt hours are required per square foot of anode surface.

The following examples are given to illustrate the invention, but are not deemed limitative of it.

#### EXAMPLE 1

Three SAE-1020 panels,  $1\frac{1}{2}$  by  $1\frac{1}{2}$  by .050 inch were cleaned in 20% HCl until all surface oxides were removed. The panels were then rinsed in water and placed in a steel beaker containing a solution of 39 g. of



40 g. of NaOH, and enough water to make 1 liter of solution. Each of the panels was used as the anodic terminal and the steel beaker was used as the cathodic terminal of a source of direct current. The temperature of the solution was maintained at 180° F., and 144 amperes per square foot was applied at a potential of 4 volts. At the termination of the 4 minutes, the panels were covered with a uniform red barium ferrate film. These filmed panels were rinsed, dried, and placed in a closed atmosphere containing 0.05% sulfur dioxide, alongside identical uncoated panels. The sulfur oxide was produced by decomposing sodium pyrosulfite with acid. The coated and uncoated test specimens were maintained in this atmosphere at 40° C. for 24 hours. The coated panels showed only the slightest evidence of corrosion, whereas the uncoated panels showed severe corrosion.

The above procedure was repeated using cast iron and 314 stainless steel panels. The results obtained were the same as will the SAE-1020 steel panels.

#### EXAMPLE 2

Steel panels, identical to those of Example 1,  $1\frac{1}{2}$  by  $1\frac{1}{2}$  by .050 inch were cleaned in 20% HCl until all surface oxides were removed. These panels were removed and placed in steel beakers containing the solutions set forth in Table I. The panel was used as the anodic terminal, and the steel beaker was used as the cathodic terminal of a source of direct current. The temperature of the solutions, the voltage, and the amperage are given in Table I. The coated panels were subjected to microscopic examination to determine the extent of any microscopic pores or breaks in the uniform surface of the coating. The results are given in Table I.

Table I

| Solution components |        | Volts | a.s.f. | Tempera-ture, °F. | Time, min. | Microscopic examination |
|---------------------|--------|-------|--------|-------------------|------------|-------------------------|
| Ba(OH) <sub>2</sub> | NaOH   |       |        |                   |            |                         |
| 1 N                 |        | 2     | 3.6    | 178               | 4          | Few pits.               |
| 1 N                 | 0.5 N  | 2     | 3.6    | 176               | 4          | Few pits.               |
| 1 N                 | 1.0 N  | 2     | 5.8    | 180               | 4          | Few pits.               |
| 1 N                 | 2 N    | 2     | 8.6    | 180               | 4          | Few pits.               |
| 1 N                 | 3 N    | 2     | 5.8    | 179               | 4          | Very few pits.          |
| 1 N                 | 5 N    | 2     | 8.6    | 180               | 4          | Very few pits.          |
| 1 N                 | 7.5 N  | 2     | 10.0   | 180               | 4          | Very few pits.          |
| 1 N                 | 10 N   | 2     | 7.2    | 178               | 4          | Very few pits.          |
| 1 N                 | 12.5 N | 2     | 11.0   | 180               | 4          | Few pits.               |
| 1 N                 | 15 N   | 2     | 7.2    | 180               | 4          | Many pits.              |

## 5

### EXAMPLE 3

The procedure of Example 2 was repeated, using different potentials for comparison. The conditions of operation are given in Table II. The coated panels were subjected to microscopic examination, and were also tested for corrosion resistance conducted under the conditions given below. The results of these tests are given in Table II.

#### $\text{SO}_2$ VAPOR CORROSION

The coated panels were suspended in a closed dessicator containing 0.05% sulfur dioxide. This quantity of sulfur dioxide was produced by the reaction of 0.025 g. of sodium pyrosulfite with sulfuric acid. The test specimens were maintained at 40° C. and 100% R.H. for 24 hours in this simulated industrial atmosphere.

#### HUMIDITY TEST

Coated panels were suspended in a dessicator kept at 100% relative humidity at 40° C. Test panels were inspected after 48 hours exposure.

#### WATER IMMERSION TEST

Coated panels were immersed in individual beakers containing distilled water at a pH of  $7.0 \pm 0.2$ . Solutions were kept at ambient temperature for 48 hours.

*Table II*

| Solution Compounds   |      | Volts | a.s.f. | Corrosion Tests     |                            |                                | Microscopic examination |
|----------------------|------|-------|--------|---------------------|----------------------------|--------------------------------|-------------------------|
|                      |      |       |        | $\text{SO}_2$ Vapor | $\text{H}_2\text{O}$ Vapor | $\text{H}_2\text{O}$ Immersion |                         |
| Ba (OH) <sub>2</sub> | NaOH |       |        |                     |                            |                                |                         |
| 1 N                  | 1 N  | 4     | 140    | Good                | Good                       | Poor                           | Numerous pores.         |
| 1 N                  | 1 N  | 4     | 130    | Good                | Good                       | Poor                           | Numerous pores.         |
| 1 N                  | 1 N  | 2     | 15     | E*                  | E*                         | E*                             | Very few pores.         |
| 1 N                  | 1 N  | 2     | 15     | E*                  | E*                         | E*                             | Very few pores.         |

\*Excellent.

While the barium ferrate coatings as obtained in the preceding examples are found to be excellent corrosion resistant films, it has been determined that after-treatments are capable of improving the corrosion resistance of the film. In particular, an after-treatment dip of the ferrous metal coated with the BaFeO<sub>4</sub> film in a dilute dichromate solution, materially increases the corrosion resistance of the coating. The dichromate, and preferably sodium dichromate, can be employed in aqueous solutions as low as about 0.2% by weight. Higher amounts can be employed if desired with the same beneficial effect.

### EXAMPLE 4

Several panels of SAE-1020 steel were coated with a BaFeO<sub>4</sub> film by anodic deposition. The films were formed by applying a potential of 2 volts at 10.5 (a.s.f.) for a period of 4 minutes. The electrolyte contained 1 N Ba(OH)<sub>2</sub> plus 5 N Na(OH) and was maintained at 95° C. One half of these coated panels were then subjected to an after-treatment by immersion for 30 seconds in a 0.2% by weight aqueous solution of sodium dichromate maintained at 50° C. The solution was neutralized to a pH of 7.0 just prior to the after-treatment. At the conclusion of the after-treatment, both the treated and untreated samples were immersed in individual beakers of distilled water at a pH of  $7.0 \pm 0.2$ , and at ambient temperatures. The time required for the appearance of a  $\frac{1}{4}$  inch diameter corrosion spot was considered as the time of failure. The untreated samples required 50 hours to fail, whereas the after-treated samples required 200 hours to fail.

The barium ferrate coatings, in addition to being good corrosion resistant films, also have been found suitable as base coatings for finish coatings of paint, lacquer or

enamel. The barium ferrate coating acts as an intermediate bonding layer, and effectively binds surface coatings such as paints, to the base metal more tenaciously than if the paint were applied directly to the metal surface. In addition, when organic enamel is applied as a finish coat over a primer coating of barium ferrate, the ferrate coating is not deleteriously effected by the baking operation which is required to yield an enamel having a hard, smooth surface.

10 Pursuant to the requirements of the patent statutes, the principle of this invention has been explained and exemplified in a manner so that it can be readily practiced by those skilled in the art, such exemplification including what is considered to represent the best embodiment of 15 the invention. However, it should be clearly understood that, within the scope of the appended claims, the invention may be practiced by those skilled in the art, and having the benefit of this disclosure, otherwise than as 20 specifically described and exemplified herein.

20 What is claimed is:

1. The process of coating the surface of a ferrous metal with a corrosion resistant coating of barium ferrate which comprises immersing said ferrous metal in an alkaline solution containing from about 0.5 N to about 7.5 N 25 of an alkali metal hydroxide and barium ions in amounts

of from about  $\frac{1}{20}$  N up to the solubility limit of barium ions in said alkaline solution, said alkaline solution having a pH of at least about 12.5, passing an electric current having a potential of at least 1.4 volts and in an amount of at least 2 amperes per square foot of ferrous metal surface through said ferrous metal, said alkaline solution serving as the electrolyte, said ferrous metal serving as the anode, and a conductor which is resistant to the electrolyte serving as the cathode.

45 2. The process of coating the surface of a ferrous metal with a corrosion resistant coating of barium ferrate which comprises immersing said ferrous metal in an alkaline solution containing barium ions in amounts of from about  $\frac{1}{20}$  N to about 1 N and an alkali metal hydroxide in

50 amounts of from about 0.5 N to about 7.5 N, said alkaline solution having a pH of at least about 12.5, passing an electric current having a potential of at least 1.4 volts and in an amount of at least 2 amperes per square foot of ferrous metal surface through said ferrous metal, said alkaline solution serving as the electrolyte, said ferrous metal serving as the anode, and a conductor which is resistant to the electrolyte serving as the cathode.

60 3. The process of claim 2 wherein the barium ions are supplied by adding barium hydroxide.

55 4. Process of claim 2 wherein said electric current has a potential of about 1.4 to 4 volts and is applied at the rate of 5 to 20 amperes per square foot of ferrous metal surface.

70 5. Process of claim 2 wherein said solution contains barium hydroxide in a concentration of about 1 N and an alkaline metal hydroxide in concentrations of about 0.5 N to 7.5 N.

65 6. The process of claim 2 wherein said ferrous metal coated with said barium ferrate is after-treated by being dipped in an aqueous solution of sodium dichromate con-

taining at least about 0.2% by weight sodium dichromate.

7. Process of coating the surface of a ferrous metal with a corrosion resistant coating of barium ferrate which comprises immersing said ferrous metal in a solution containing about 1 N barium hydroxide and about 5 N of an alkaline metal hydroxide, said solution having a pH of at least 12.5, passing an electric current through said ferrous metal, said current having a potential of about 1.4 to about 2 volts and being applied at a rate between 5 to 20 amperes per square foot of ferrous metal surface, said solution serving as an electrolyte, said ferrous metal serving

as the anode, and a conductor which is resistant to the electrolyte serving as the cathode.

### References Cited by the Examiner

## FOREIGN PATENTS

692,124 6/40 Germany.

JOHN H. MACK, *Primary Examiner.*

10 JOSEPH REBOLD, *Examiner.*

UNITED STATES PATENT OFFICE  
CERTIFICATE OF CORRECTION

Patent No. 3,206,384

September 14, 1965

Paul H. Margulies et al.

It is hereby certified that error appears in the above numbered patent requiring correction and that the said Letters Patent should read as corrected below.

Column 1, line 65, for "one-formation" read -- one-step formation --; column 2, line 55, for "exceeded" read -- exceed --; column 3, line 14, for "Flms" read -- Films --; line 36, for "then" read -- than --; column 6, line 45, for "last" read -- least --.

Signed and sealed this 9th day of August 1966.

(SEAL)

Attest:

ERNEST W. SWIDER

Attesting Officer

EDWARD J. BRENNER

Commissioner of Patents